# EUROPEAN PATENT SPECIFICATION

(11) **EP 0 421 740 B1**
(45) Date of publication and mention of the grant of the patent: **06.08.1997**
(21) Application number: 90310790.2
(22) Date of filing: 02.10.1990
(51) Int. Cl.: G03C 1/035, G03C 1/015

(54) **Silver halide photographic light-sensitive material with high-sensitivity and improved fog and granularity and method of its production**
Silberhalogenid photographisches lichtempfindliches Material mit hoher Empfindlichkeit und verbessertem Schleier und Körnigkeit und sein Herstellungsverfahren
Matériau photographique à l'halogénure d'argent sensible à la lumière à haute sensibilité et voile et granularité améliorés, et méthode pour sa fabrication

(30) Priority: 03.10.1989 JP 259309/89
(43) Date of publication of application: 10.04.1991
(73) Proprietor: KONICA CORPORATION, Tokyo 160 (JP)
(72) Inventor: Yagi, Toshihiko, Konica Corporation, Tokyo (JP); Hoshino, Hiroyuki, Konica Corporation, Tokyo (JP); Kondou, Toshiya, Konica Corporation, Tokyo (JP); Heki, Katsuhiko, Konica Corporation, Tokyo (JP); Suzuki, Katsuhiko, Konica Corporation, Tokyo (JP)
(74) Representative: Simpson, Alison Elizabeth Fraser

(56) References cited:
- EP-A- 0 165 576
- EP-A- 0 273 411
- DE-A- 3 707 135
- FR-A- 2 281 592
- JP-A- 6 114 630

## Description

### FIELD OF THE INVENTION

The present invention relates to a silver halide photographic light-sensitive material and a method of its production, more specifically to a light-sensitive material with high sensitivity, reduced and excellent granularity and a production method thereof.

### BACKGROUND OF THE INVENTION

In recent years, there have been increasing demands for improvements in the sensitivity and image quality of silver halide photographic light-sensitive materials.

In response to these demands, there have been proposed various methods for controlling a shape, a size distribution and a composition of a silver halide grain.

Japanese Patent Publication Open to Public Inspection No. 113934/1983 discloses a method of improving color photographic light-sensitive materials wherein a tabular silver halide emulsion having a diameter/thickness ratio of a grain (aspect ratio) exceeding 8 is applied to a green or red-sensitive layer.

However, the emulsions having high aspect ratios exceeding 8 does not have satisfactory improvement in sensitivity or granularity since its latent image-forming efficiency is not necessarily high while having an excellent photoreceptive efficiency.

Further, investigations have been made to prepare core/shell type tabular grains having a high silver iodide content phase in the core as well as to increase a monodispersion degree thereof.

Japanese Patent Publication Open to Public Inspection (hereinafter referred to as Japanese Patent O.P.I. Publication) Nos. 14636/1986, 112142/1986 and 163451/1988 disclose monodispersed twinned tabular grains having a core-shell structure.

In the above disclosures, the grains having the aspect ratios of 3 to 8 show good performance but have insufficient improvement in sensitivity and granularity.

### SUMMARY OF THE INVENTION

The object of the present invention is to provide a silver halide photographic light sensitive material (hereinafter referred to as a light-sensitive material) with high sensitivity, improved fog and excellent granularity and a production method thereof, more specifically to a light-sensitive material containing an improved core/shell type twinned silver halide grains and a production method thereof.

The above object of the invention is accomplished by a silver halide photographic light-sensitive material comprising a support and provided thereon photographic component layers including at least one light-sensitive emulsion layer containing a monodispersed silver halide emulsion consisting mainly of twined halide grains, characterised in that the silver halide grains comprise: (a) a high silver iodide core; (b.) an aspect ratio of not less than 1.3 to less than 2; (c.) mainly [111] planes; and (d.) parralel twin planes of an even number in a ratio of 50% or more by number based on the total twinned grains.

### BRIEF DESCRIPTION OF THE DRAWINGS

Figs. 1 and 2 are X ray diffraction patterns at (420) of emulsions Em-1 and emulsion Em-2 prepared in Examples 2 and 4, respectively, both having two peaks corresponding to high and low silver iodide contents.

Fig. 3 is a schematic diagram of the twinned silver halide grain of the present invention, in which a-a', b-b' and c-c' each represent parallel twinned planes. (A) and (B) show twinned crystals comprising {111} planes alone, and (C) shows a twinned crystal comprising about 95% {111} planes and about 5% {100} planes.

### DETAILED DESCRIPTION OF THE INVENTION

It has been found that improvements in sensitivity and image quality can be accomplished with an emulsion having such a low aspect ratio as described above, while emulsions having higher aspect ratios are popular.

In the present invention, a monodispersion of a silver halide emulsion is defined by that the silver halide grains falling within the range of 80 to 120% of an average grain diameter $\overline{\text{d}}$ accounts for not less than 70%, preferably not less than 80%, more preferably not less than 90% by weight of the total silver halide grains.

The average grain size $\overline{\text{d}}$ is defined by the grain size di in which the product of ni x di³ is maximized, wherein ni is the number of the grains having the size di (the significant figure is calculated down to the third decimal place and the forth digit is rounded to the nearest whole number).

A diameter of a twinned grain is defined by a diameter of the circle having the same area as that of the projected grain.

Grain size can be determined by taking an electron micrograph of the grain at a magnifying rate of 10000 to 50000 and measuring the diameters of the printed grain images or the area of the projected images of more than 1000 grains selected arbitrarily.

The silver halide emulsion used in the invention has a monodispersion degree of not more than 20%, preferably not more than 15%, wherein the monodispersion degree is defined by the following equation:$\text{(standard deviation of grain size/average grain size) x 100} \text{= monodispersion degree (%)}$

The grain size is determined by the method described above, and the average grain size is a simple average value calculated by the following equation:$\text{average grain size = Σdini/Σni}$

In the invention, the silver halide emulsion is prepared preferably by precipitating a high iodide content phase on a monodispersed seed grain, more preferably by the method described in Japanese Patent O.P.I. Publication No. 6643/1986, in which monodispersed, twinned spherical seed grains are grown. The silver halide emulsion of the invention has mainly an even number of parallel twinned planes, preferably two twinned planes.

The silver halide emulsion of the invention comprises a silver iodobromide having an average silver iodide content of 4 to 20 mol%, preferably 5 to 15 mol%.

The concentration of an aqueous solution of silver nitrate used to grow the high silver iodide content phase present in the center of a grain is not more than 1 N, preferably 0.3 to 0.8 N.

The twinned silver halide grains of the invention comprise mainly {111} planes in a ratio of not less than 60%, preferably 70 to 100%, more preferably 75 to 98% based on the whole grain.

The average ratio of a diameter of a circle having the same area as that of the projected major plain to a distance (thickness) between two grain surfaces parallel to the twinned planes (aspect ratio) is less than 1.3 to less than 2.0.

The method of producing a silver halide emulsion of the invention by adding an aqueous silver salt solution and an aqueous halide solution in the presence of protective colloid is characterized by taking the following steps:
(a) forming nuclear grains having a silver iodide content of 0 to 5 mol% while pBr of the mother liquid is maintained at 2.0 to -0.7 during at least the first half of the time necessary for forming the nuclear grains;
(b) forming monodispersed seed grains of a spherical twinned crystal by ripening the nuclear grains in the presence of a silver halide solvent of 10⁻⁵ to 2.0 mol per mol silver halide; and
(c) growing the seed grains by adding the water-soluble silver salt and halide solutions and/or fine silver halide grains.

The two or more twinned planes may be or may not be parallel to each other. The grains may comprise {111} planes, {100} planes or combination thereof.

In the formation of the nuclear grains, pBr is maintained at -0.7 to 2.0, preferably -0.7 to 1.5 during at least a half of the time necessary for forming the grains.

The nuclear grains may be monodispersed or polydispersed. Polydispersion is defined by the monodispersion degree of not less than 25%. The nuclear grains contain twinned grains in a ratio of not less than 50%, preferably not less than 70%, and more preferably not less than 90% based on the total grains.

Substantially monodispersed spherical grains are prepared by adding the silver salt and halide solutions to the nuclear grains in the presence of a silver halide solvent of 10⁻⁵ to 2.0 mol per mol silver halide. Substantially monodispersed grains are defined by the grains having the monodispersion degree of less than 25%.

Substantially spherical grains are defined by the grains which are round to such extent that {111} and {100} planes are not clearly recognizable via electron micrographic observation and have a L/ℓ ratio of 1.0 to 2.0, preferably 1.0 to 1.5, wherein L and ℓ represent the maximum and minimum grain diameters, respectively.

The spherical grains account for not less than 60%, preferably not less than 80%, and more preferably almost all of the total seed grains.

Examples of the silver halide solvent used in the seed grain formation are (a) organic thioethers described in US Patent Nos. 3,271,157, 3,531,289 and 3,574,628, Japanese Patent O.P.I. Publication Nos. 1019/1979 and 158917/1979 and Japanese Patent Examined Publication No. 30571/1983; (b) thiourea derivatives described in Japanese Patent O.P.I. Publication Nos. 82408/1978, 29829/1980 and 77737/1980; (c) AgX solvents having a thiocarbonyl group located between an oxygen or sulfur atom and a nitrogen atom described in Japanese Patent O.P.I. Publication Nos. 144319/1978; (d) imidazoles described in Japanese Patent Publication No. 100717/1979; (e) sulfites; (f) thiocyanates, (g) ammonia; (h) hydroxylalkyl-substituted ethylenediamines described in Japanese Patent O.P.I. Publication No. 196228/1982; (i) substituted mercaptotetrazoles described in Japanese Patent O.P.I. Publication No. 202531/1982; (j) water-soluble bromides; and (k) benzimidazole derivatives described in Japanese Patent O.P.I. Publication No. 54333/1983.

Examples of these silver halide solvents (a) to (k) are given below.

(e) K₂SO₃, Na₂SO₃

(f) NH₄SCN, KSCN

(g) NH₃

(j) NaBr, NH₄Br, KBr

These solvents may be used in combination. Preferred solvents are thioethers, thiocyanates, thioureas, ammonia and bromides, more preferably a combination of ammonia and bromide.

pH is 3 to 13, preferably 6 to 12, and the temperature is 30 to 70°C, preferably 35 to 50.

In one mode of preferred embodiment of the present invention, the seed grains are prepared by ripening for 30 seconds to 10 minutes using 0.4 to 1.0 mol/ℓ ammonia and 0.03 to 0.5 mol/ℓ potassium bromide in combination at pH of 10.8 to 11.2 and a temperature of 35 to 45°C.

A water-soluble silver salt may be added for adjustment of ripening during the seed grain formation.

The seed grains are grown by adding the silver salt and halide solutions by the double jet method with the addition speed varied gradually so that the new grains are not formed and Ostwald ripening does not occur, as described in Japanese Patent O.P.I. Publication Nos. 39027/1976, 142329/1980, 113928/1983, 48521/1979 and 49938/1983. The seed grains can be grown by another method described in the proceeding of the 1983 annual meeting of the Society of Photographic Science and Technology of Japan, p. 88, in which fine silver halide grains coexist in the emulsion for recrystallization on the nuclear grains.

In the preparation of the high silver iodide content silver halide emulsion of the present invention, pAg is maintained at 5 to 11, preferably 6.0 to 9.5; the temperature is 40 to 85°C, preferably 60 to 80°C; and pH is 1.5 to 5.8, preferably 1.8 to 3.0.

In the present invention, a stirring condition is an important factor. The stirring apparatus disclosed in Japanese Patent O.P.I. Publication No. 160123/1988 is preferably used, in which a nozzle for adding a solution is placed near the mother liquid inlet so that the nozzle is dipped in the liquid. It is preferable that the rotating rate of the stirrer be 400 to 1200 rpm.

The silver halide emulsion used in the present invention may be subjected to chemical sensitization by an ordinary method and to spectral sensitization to the prescribed wavelength regions with sensitizing dyes.

The silver halide emulsion may contain an antifogging agent, a stabilizer and other additives. Gelatin is preferably used as a binder.

The emulsion layers and other hydrophilic colloid layers may be hardened and contain a plasticizer and a latex.

The present invention is applied preferably to color photographic light-sensitive materials such as color negative films and color reversal films.

The emulsion layers of the color photographic light-sensitive materials contain couplers.

There may be added a colored coupler having a corrective effect, a competitive coupler and a compound that releases photographically useful fragments such as a development accelerator, a bleaching accelerator, a developer, a silver halide solvent, a toning agent, a hardener, a fogging agent, an antifogging agent, a chemical sensitizer, a spectral sensitizer and a desensitizer by coupling with the oxidation product of a developing agent.

The light-sensitive material may be provided with supplementary layers such as a filter layer, an antihalation layer and an anti-irradiation layer. These layers and/or emulsion layers may contain a dye that elutes from the light-sensitive material or is bleached during development.

The light-sensitive material may contain a formalin scavenger, a fluorescent brightening agent, a matting agent, a lubricant, an image stabilizer, a surfactant, an anti-fogging agent, a development accelerator, a development retarder and a bleaching accelerator.

Examples of the supports are polyethylene-laminated paper, polyethylene terephthalate film, baryta paper and cellulose triacetate film.

The light-sensitive material is subjected to conventional processing after exposure.

### EXAMPLE

The present invention is hereinafter described in more detail by means of the following examples.

### Example 1

### Preparation of spherical seed emulsion

A monodispersed spherical seed emulsion was prepared by the method described in Japanese Patent O.P.I. Publication No. 6643/1986.

| Solution A₁ | |
|---|---|
| Ossein gelatin | 150 g |
| Potassium bromide | 53.1 g |
| Potassium iodide | 24 g |
| Water was added to the total quantity of 7.2 ℓ. | |

| Solution B₁ | |
|---|---|
| Silver nitrate | 1.5 kg |
| Water was added to the total quantity of 6ℓ. | |

| Solution C₁ | |
|---|---|
| Potassium bromide | 1327 g |
| 1-phenyl-5-mercaptotetrazole in methanol solution | 0.3 g |
| Water was added to the total quantity of 3ℓ. | |

| Solution D₁ | |
|---|---|
| Aqueous ammonia (28%) | 705 mℓ |

To solution A₁ stirred vigorously at 40°C, solutions B₁ and C₁ were added by the double jet method at pBr of 1.09 to 1.15 in 30 seconds to prepare nuclear grains.

One minute and 30 seconds later, solution C₁ was added in 20 seconds, followed by ripening for 5 minutes, wherein the KBr and ammonia concentrations were 0.071 mol/ℓ and 0.63 mol/ℓ, respectively.

Then, pH was adjusted to 6.0, and the emulsion was immediately desalted and washed with water. Observation via an electron microscope revealed that this seed emulsion contained the monodispersed spherical grains having an average grain size of 0.36 µm and a monodispersion degree of 18%.

### Example 2

### Preparation of emulsion of the present invention

An emulsion of the present invention having an average silver iodide content of 6.0% was prepared as follows:

| Solution A₂ | |
|---|---|
| Ossein gelatin | 76.8 g |
| Seed emulsion of Example 1 | 0.191 mol eq. |
| Water was added to the total quantity of 4ℓ. | |

| Solution B₂₋₁ | |
|---|---|
| Silver nitrate | 206.4 g |
| Water was added to the total quantity of 2209 mℓ. | |

| Solution C₂₋₁ | |
|---|---|
| Ossein gelatin | 88.4 g |
| Potassium bromide | 101.2 g |
| Potassium iodide | 60.5 g |
| Water was added to the total quantity of 2209 mℓ. | |

| Solution B₂₋₂ | |
|---|---|
| Silver nitrate | 961.2 g |
| Water was added to the total quantity of 5143 mℓ. | |

| Solution C₂₋₂ | |
|---|---|
| Ossein gelatin | 179 g |
| Potassium bromide | 667 g |
| Potassium iodide | 9.4 g |
| Water was added to the total quantity of 3800 mℓ. | |

Each six nozzles for supplying the B₂ and C₂ solutions were disposed under a stirring propeller of the mixing apparatus disclosed in Japanese Patent O.P.I. Publication No. 160128/1988.

Solutions B₂₋₁ and C₂₋₁ were added to solution A₂ stirred at a high speed of 1000 rpm at 75°C by the double jet method with an addition rate increased gradually from 8.57 mℓ/min at the beginning to 24.16 mℓ/min at the final stage over a period of 135 minutes, during which pAg and pH were maintained at 8.0 and 2.0, respectively.

Subsequently, solutions B₂₋₂ and C₂₋₂ were added by the double jet method over a period of 73.5 minutes. The initial and final addition rates of solution B₂₋₂ were 43.1 mℓ/min and 97.0 mℓ/min, respectively, and the initial and final addition rates of solution C₂₋₂ were 31.8 mℓ/min and 71.6 mℓ/min, respectively.

pAg and pH were maintained at 9.0 and 2.0 during the addition.

After completion of the addition, pH was adjusted to 6.0, and the emulsion was desalted by a conventional method.

Observation via an electron microscope revealed that the grains were monodispersed and 100% twinned and that the monodispersion degree was 13% and the ratio of the grains having twinned planes of an even number was 85%. Measurement by X ray diffraction revealed that the grains had two peaks and that there existed a clear border between a high silver iodide content phase (core) and a low silver iodide content phase.

The grains were found to comprise mainly {111} planes.

The average aspect ratio of the grains having an even number of twinned planes was 1.9. This emulsion is designated as Em-1.

### Example 3

### Preparation of spherical seed emulsion

A monodispersed spherical seed emulsion having an average grain size of 0.34 µm and a monodispersion degree of 21% was prepared in the same manner as in Example 1 except that ripening time was changed from 5 minutes to 1 minute.

### Example 4

An emulsion of the present invention having an average silver iodide content of 6.0 mol% was prepared as follows:

| Solution A₄ | |
|---|---|
| Ossein gelatin | 74.1 g |
| Seed emulsion of Example 3 | 0.306 mol eq. |
| Water was added to the total quantity of 4000 mℓ. | |

| Solution B₄₋₁ | |
|---|---|
| Silver nitrate | 206.4 g |
| Nitric acid (1.38) | 5.5 mℓ |
| Water was added to the total quantity of 1105 mℓ. | |

| Solution C₄₋₁ | |
|---|---|
| Ossein gelatin | 44.2 g |
| Potassium bromide | 101 g |
| Potassium iodide | 60.8 g |
| Water was added to the total quantity of 1105 mℓ. | |

| Solution B₄₋₂ | |
|---|---|
| Silver nitrate | 941 g |
| Nitric acid (1.38) | 6.6 mℓ |
| Water was added to the total quantity of 1582 mℓ. | |

Using the same apparatus as in Example 2, an emulsion was prepared.

To solution A₄ stirred at a high speed of 1000 rpm at 75°C, solutions B₄₋₁ and C₄₋₁ were added by the double jet method. The initial and final addition rates were 12.21 mℓ/min and 26.03 mℓ/min, respectively, and the addition time was 58 minutes. pAg and pH were maintained at 8.0 and 2.0, respectively, during the addition.

Then, solutions B₄₋₂ and C₄₋₂ were added by the double jet method. The initial and final addition rates were 19.44 mℓ/min and 44.0 mℓ/min, respectively, and the addition time was 50 minutes. pAg and pH were maintained at 8.0 and 2.0, respectively during the addition. After completion of addition, pH was adjusted to 6.0, followed by desalting and washing.

Observation via an electron microscope revealed that the grains were monodispersed and 100% twinned and that a monodispersion degree was 14% and the ratio of the grains having twinned planes of an even number was 82%. The grains having an even number of twinned planes consisted of 95% {111} planes and 5% {100} planes. The average aspect ratio of the grains having an even number of twinned planes was 1.7.

Measurement by X ray diffraction revealed that the grains had two peaks corresponding to a high silver iodide content phase (core) and a low silver iodide content phase and that there existed a clear border between the two phases.

This emulsion is designated as Em-2.

### Example 5

Silver ioidobromide emulsion Em-3 having an average silver iodide content of 9.0% was prepared in the same manner as in Example 4 except that the volume of the high iodide content phase was increased.

Em-3 consisted of 100% twinned grains having a monodispersion degree of 14% and the ratio of the grains having twinned planes of an even number was 80%. The grains having an even number of twinned planes had an average aspect ratio of 1.9 and consisted of 93% {111} planes and 7% {100} planes.

### Example 6

The layers having the following compositions were formed on a triacetyl cellulose film support in the order from the support to prepare comparative light-sensitive material sample No. 1.

In the examples below, the addition amounts are expressed in grams per m² unless otherwise stated. The amounts of silver halide and colloid silver are converted to silver, and those of sensitizing dyes are expressed in mole per mol of silver.

| Layer 1: Antihalation layer | |
|---|---|
| Black colloidal silver | 0.2 |
| Gelatin | 0.4 |
| UV absorber UV-1 | 0.3 |
| High boiling organic solvent Oil-1 | 0.3 |

| Layer 2: Interlayer | |
|---|---|
| Gelatin | 1.0 |

| Layer 3: First red-sensitive emulsion layer | |
|---|---|
| Silver iodobromide emulsion (AgI 7 mol%, octahedron, 0.3 µm) | 0.6 |
| Gelatin | 1.2 |
| Sensitizing dye S-1 | 8 x 10⁻⁴ |
| Sensitizing dye S-2 | 5 x 10⁻⁴ |
| Sensitizing dye S-3 | 3 x 10⁻⁵ |
| Coupler C-1 | 0.10 |
| Coupler C-3 | 0.25 |
| Colored coupler CC-1 | 0.04 |
| DIR coupler D-2 | 0.05 |
| High boiling organic solvent Oil-1 | 0.45 |

| Layer 5: Third red-sensitive emulsion layer | |
|---|---|
| Em-A shown below | 1.6 |
| Gelatin | 1.6 |
| Sensitizing dye S-1 | 1 x 10⁻⁴ |
| Sensitizing dye S-2 | 1 x 10⁻⁴ |
| Sensitizing dye S-3 | 1 x 10⁻⁵ |
| Coupler C-1 | 0.20 |
| Coupler C-2 | 0.10 |
| Colored coupler CC-1 | 0.02 |
| DIR coupler D-2 | 0.05 |
| High boiling organic solvent Oil-1 | 0.40 |

| Layer 6: Interlayer | |
|---|---|
| Gelatin | 0.80 |
| Additive SC-1 | 0.03 |
| Additive SC-2 | 0.02 |
| High boiling organic solvent Oil-2 | 0.05 |

| Layer 7: First green-sensitive emulsion layer | |
|---|---|
| Silver iodobromide emulsion (AgI 7 mol%, octahedron, 0.3 µm) | 0.4 |
| Gelatin | 0.8 |
| Sensitizing dye S-4 | 6 x 10⁻⁴ |
| Sensitizing dye S-5 | 1 x 10⁻⁴ |
| Sensitizing dye S-6 | 1 x 10⁻⁴ |
| Coupler M-1 | 0.05 |
| Coupler M-3 | 0.25 |
| Colored coupler CM-1 | 0.04 |
| DIR coupler D-1 | 0.06 |
| High boiling organic solvent Oil-2 | 0.40 |

| Layer 8: Second green-sensitive emulsion layer | |
|---|---|
| Silver iodobromide emulsion (AgI 8 mol%, octahedron, 0.7 µm) | 0.8 |
| Gelatin | 1.1 |
| Sensitizing dye S-4 | 3 x 10⁻⁴ |
| Sensitizing dye S-5 | 5 x 10⁻⁵ |
| Sensitizing dye S-6 | 5 x 10⁻⁵ |
| Coupler M-1 | 0.05 |
| Coupler M-3 | 0.20 |
| Colored coupler CM-1 | 0.03 |
| DIR coupler D-1 | 0.05 |
| High boiling organic solvent Oil-2 | 0.30 |

| Layer 9: Third green-sensitive emulsion layer | |
|---|---|
| Em-A | 1.2 |
| Gelatin | 1.1 |
| Sensitizing dye S-4 | 2 x 10⁻⁴ |
| Sensitizing dye S-5 | 5 x 10⁻⁴ |
| Sensitizing dye S-6 | 5 x 10⁻⁴ |
| Coupler M-2 | 0.05 |
| Coupler M-3 | 0.10 |
| Colored coupler CM-1 | 0.02 |
| DIR coupler D-1 | 0.02 |
| High boiling organic solvent Oil-2 | 0.30 |

| Layer 10: Yellow filter layer | |
|---|---|
| Yellow colloidal silver | 0.05 |
| Gelatin | 1.0 |
| Additive SC-1 | 0.03 |
| Additive SC-2 | 0.02 |
| High boiling organic solvent Oil-2 | 0.05 |

| Layer 11: First blue-sensitive emulsion layer | |
|---|---|
| Silver iodobromide emulsion (AgI 7 mol%, octahedron 0.7 µm) | 0.20 |
| Gelatin | 1.30 |
| Sensitizing dye S-7 | 1 x 10⁻³ |
| Coupler Y-1 | 0.80 |
| DIR coupler D-2 | 0.10 |
| High boiling organic solvent Oil-2 | 0.28 |

| Layer 12: Second blue-sensitive emulsion layer | |
|---|---|
| Silver iodobromide emulsion (AgI 8 mol%, octahedron, 0.7 µm) | 0.50 |
| Gelatin | 0.50 |
| Sensitizing dye S-7 | 5 x 10⁻⁴ |
| Coupler Y-1 | 0.60 |
| DIR coupler D-2 | 0.08 |
| High boiling organic solvent Oil-2 | 0.25 |

| Layer 13: Third blue-sensitive emulsion layer | |
|---|---|
| Em-B shown below | 0.70 |
| Gelatin | 0.70 |
| Sensitizing dye S-7 | 2 x 10⁻⁴ |
| Coupler Y-1 | 0.20 |
| DIR coupler D-2 | 0.01 |
| High boiling organic solvent Oil-2 | 0.07 |

| Layer 14: First protective layer | |
|---|---|
| Silver iodobromide (AgI 1 mol%, 0.08 µm) | 0.3 |
| Gelatin | 1.0 |
| UV absorber UV-1 | 0.1 |
| UV absorber UV-2 | 0.1 |
| Formalin scavenger HS-1 | 0.5 |
| Formalin scavenger HS-2 | 0.2 |
| High boiling organic solvent Oil-1 | 0.1 |
| High boiling organic solvent Oil-3 | 0.1 |

| Layer 15: Second protective layer | |
|---|---|
| Gelatin | 0.7 |
| Alkali-soluble matting agent (average grain size: 2 µm) | 0.12 |
| Polymethyl methacrylate (average grain size: 3 µm) | 0.02 |
| Lubricant WAX-1 | 0.04 |
| Antistatic agent Su-1 | 0.004 |

In addition to these compositions, each layer contained coating aid Su-2, dispersion aids Su-2 and Su-3, hardeners H-1 and H-2, stabilizer Stab-1, antifogging agents AF-1 and AF-2 and preservative DI-1.

### Em-A:

A monodispersed octahedral silver iodobromide emulsion having an average AgI content of 6 mol%, a high silver iodide content phase in the core, a monodispersion degree of 13% and an average grain size of 1.0 µm.

### Em-B:

A monodispersed octahedral silver iodobromide emulsion having an average AgI content of 9 mol%, a high silver iodide content phase in the core, a monodispersion degree of 14% and an average grain size of 1.0 µm.

### Em-C:

A tabular silver iodobromide emulsion having an average AgI content of 6 mol%, a high silver iodide content phase in the core, a monodispersion degree of 21%, an average aspect ratio of 6 and an average grain size of 1.8 µm.

### Em-D:

A tabular silver iodobromide emulsion having an average AgI content of 9 mol%, a high silver iodide content phase in the core, a monodispersion degree of 19%, an average aspect ratio of 5 and an average grain size of 1.6 µm.

The comparative light-sensitive material sample No. 2 was prepared in the same manner as in sample No. 1 except that Em-A and Em-B used in Layers 5, 9 and 13 were replaced with Em-C and Em-D as shown in Table 1.

The inventive light-sensitive material samples No. 3 to 5 were prepared in the same manner as in comparative sample No. 1 except that the emulsions in Layers 5, 9 and 13 were replaced with Em-1, Em-2 and Em-3 of the invention each chemically sensitized with sodium thiosulfate, chloroauric acid and ammonium thiocyanate, as shown in Table 1.

Sample Nos. 1 to 5 were each subjected to wedge exposure with white light and then to following processing:

| Processes (38°C) | |
|---|---|
| Color development | 3 minutes 15 seconds |
| Bleaching | 6 minutes 30 seconds |
| Washing | 3 minutes 15 seconds |
| Fixation | 6 minutes 30 seconds |
| Stabilization | 1 minute 30 seconds |
| Drying | |

The compositions of the processing solutions used in the respective processes are as follows:

| Color developer | |
|---|---|
| 4-amino-3-methyl-N-ethyl-N-β-hydroxyethylaniline sulfate | 4.75 g |
| Sodium sulfite anhydrous | 4.25 g |
| Hydroxylamine 1/2 sulfate | 2.0 g |
| Potassium carbonate anhydrous | 37.5 g |
| Sodium bromide | 1.3 g |
| Trisodium nitrilotriacetate (monohydrate) | 2.5 g |
| Potassium hydroxide | 1.0 g |
| Water was added to the total quantity of 1ℓ (pH = 10.1). | |

Water was added to the total quantity of 1ℓ, and pH was adjusted to 6.0 with aqueous ammonia.

| Fixer | |
|---|---|
| Ammonium thiosulfate | 175.0 g |
| Ammonium sulfite anhydrous | 8.5 g |
| Sodium metabisulfite | 2.3 g |
| Water was added to the total quantity of 1ℓ, and pH was adjusted to 6.0 with acetic acid. | |

| Stabilizer | |
|---|---|
| Formalin (37% aqueous solution) | 1.5 mℓ |
| Konidax produced by Konica Corporation | 7.5 mℓ |
| Water was added to the total quantity of 1ℓ. | |

Fog and relative sensitivity of each sample were measured with blue, green and red light. Granularity (RMS) was determined by scanning an area having the density of fog + 0.3 with a microdensitometer having an opening scanning area of 250 µm2 and measuring a density variation.

The results are shown in Table 2.

As is evident from Table 2, the inventive light-sensitive materials showed remarkable improvements if fog, sensitivity and granularity in comparison with the comparative light-sensitive materials.

Of the inventive light-sensitive materials, the light-sensitive materials containing the AgX grains having {100} planes had better performance.

## Claims

1. A silver halide photographic light-sensitive material comprising
a support and provided thereon photographic component layers including
at least one light-sensitive emulsion layer containing a monodispersed silver halide emulsion consisting mainly of twinned silver halide grains,
characterised in that the silver halide grains comprise:
a. a high silver iodide core;
b. an aspect ratio of not less than 1.3 to less than 2;
c. mainly [111] planes; and
d. parallel twin planes of an even number in a ratio of 50% or more by number based on the total twinned grains.

2. The light-sensitive material of claim 1, characterised in that the twinned grains consist of [111] and [100] planes.

3. The light-sensitive material of claim 2, characterised in that 60 % or more of the twinned grains consist of [111] planes.

4. The light-sensitive material of claim 3. characterised in that 70 % to 100% of the twinned grains consist of [111] planes.

5. The light-sensitive material of claim 4, characterised in that 75 % to 98% of the twinned grains consist of [111] planes.

6. The light-sensitive material of claim 1, characterised in that the silver halide emulsion has a monodispersion degree of 20 % or less. provided that the monodispersion degree is defined by the following equation:$\text{Monodispersion degree = (standard deviation of grain size/average grain size) X 100}$

7. The light-sensitive material of claim 6. characterised in that the monodispersion degree is 15 % or less.

8. The light-sensitive material of claim 1, characterised in that the silver halide emulsion comprises silver bromoiodide grains having an average silver halide content of 4 to 20 mol %.

9. The light-sensitive material of claim 8. characterised in that the average silver halide content is 5 to 15 mol %.

10. The light-sensitive material of claim 3, characterised in that the twinned silver halide grains have two twinned planes.

11. A process for forming a light-sensitive material according to claim 1, characterised in that the silver halide grains are prepared by the following three steps:
Step 1: forming nuclear grains having a silver iodide content of 0 to 5 mol % by adding a water-soluble silver salt solution and a water-soluble halide solution to an aqueous protective colloid solution while maintaining the pBr of the mother liquid at - 0.7 to 2.0 during at least the first half of the time necessary for forming the nuclear grains;
Step 2: forming monodispersed seed grains of a twinned spherical crystal by ripening the nuclear grains in the presence of a silver halide solvent of 10⁻⁵ to 2.0 mol per mol of silver halide; and
Step 3: growing the seed grains by adding a water-soluble silver salt solution and a water-soluble halide solution, or the same in the presence of fine silver halide grains.

12. The process according to claim 11, characterised in that the pH of the mother liquid is maintained at 1.5 to 5.8 during the formation of any portion of at least 30 % by volume of the silver halide grains.

13. The process according to claim 11, characterised in that the pBr in Step 1 is maintained at - 0.7 to 1.5.

14. The process according to claim 11, characterised in that the ratio of twinned nuclear grains contained in the whole nuclear grains is 50 % or more.

15. The process according to claim 14. characterised in that the ratio is 70 % or more.

16. The process according to claim 15, characterised in that the ratio is 90 % or more.

17. The process according to claim 11, characterised in that the ratio of spherical seed grains contained in the whole seed grains is 60 % or more.

18. The process according to claim 17, characterised in that the ratio is 80 % or more.

19. The process according to claim 14, characterised in that the the silver halide solvent is at least one selected from an organic thioether, a thiourea derivative, a compound having a thiocarbonyl group between an oxygen atom or a sulfur atom and a nitrogen atom, an imidazole derivative, a sulfite salt, a thiocyanate derivative. ammonia, an ethylene diamine derivative substituted with hydroxyalkyl, a substituted mercaptotetrazole derivative, a water-soluble bromide and a benzoimidazole derivative.

20. The process according to claim 19, characterised in that the silver halide solvent is at least one selected from an organic thioether, a thiocyanate derivative, ammonia and a water-soluble bromide.

21. The process according to claim 20, characterised in that the silver halide solvent is a combination of ammonia and a water-soluble bromide.

22. The process according to claim 11, characterised in that the pH and temperature in Steps 2 and 3 are 3 to 13 and 30 to 70°C respectively.

23. The process according to claim 22, characterised in that the pH and temperature in are 6 to 12 and 30 to 70°^{C} respectively.

24. The process according to claim 11, characterised in that the pAg, temperature and pH in Step 3 are 5 to 11, 40 to 85^{°C} and 1.8 to 3.0 respectively.

25. The process according to claim 24, characterised in that the pAg, temperature and pH are 6.0 to 9.5. 60 to 80°^{C} and 1.8 to 3.0 respectively.

## Patentansprüche

1. Lichtempfindliches photographisches Silberhalogenid-Aufzeichnungsmaterial, das einen Schichtträger und darauf vorgesehene photographische Schichtkomponenten, die mindestens eine lichtempfindliche Emulsionsschicht, die eine monodisperse Silberhalogenidemulsion hauptsächlich aus Silberhalogenidzwillingskörnchen enthält, umfaßt, wobei das lichtempfindliche Aufzeichnungsmaterial dadurch gekennzeichnet ist, daß die Silberhalogenidkörnchen
a) einen Kern mit hohem Silberjodidgehalt;
b) ein Seitenverhältnis von nicht weniger als 1,3 bis weniger als 2;
c) hauptsächlich [111]-Flächen und
d) parallele Zwillingsflächen einer geraden Zahl in einem zahlenmäßigen Anteil von 50% oder mehr, bezogen auf die gesamten Zwillingskörnchen,
aufweisen.

2. Lichtempfindliches Aufzeichnungsmaterial nach Anspruch 1, dadurch gekennzeichnet, daß die Zwillingskörnchen aus [111]- und [100]-Flächen bestehen.

3. Lichtempfindliches Aufzeichnungsmaterial nach Anspruch 2, dadurch gekennzeichnet, daß 60% oder mehr der Zwillingskörnchen aus [111]-Flächen bestehen.

4. Lichtempfindliches Aufzeichnungsmaterial nach Anspruch 3, dadurch gekennzeichnet, daß 70% bis 100% der Zwillingskörnchen aus [111]-Flächen bestehen.

5. Lichtempfindliches Aufzeichnungsmaterial nach Anspruch 4, dadurch gekennzeichnet, daß 75% bis 98% der Zwillingskörnchen aus [111]-Flächen bestehen.

6. Lichtempfindliches Aufzeichnungsmaterial nach Anspruch 1, dadurch gekennzeichnet, daß die Silberhalogenidemulsion einen Monodispersionsgrad von 20% oder weniger aufweist, wobei gilt, daß der Monodispersionsgrad durch die folgende Gleichung definiert ist:$\text{Monodispersionsgrad = (Standarabweichung der Korngröße/} \text{mittlere Korngröße) x 100.}$

7. Lichtempfindliches Aufzeichnungsmaterial nach Anspruch 6, dadurch gekennzeichnet, daß der Monodispersionsgrad 15% oder weniger ist.

8. Lichtempfindliches Aufzeichnungsmaterial nach Anspruch 1, dadurch gekennzeichnet, daß die Silberhalogenidemulsion Silberbromjodidkörnchen mit einem mittleren Silberhalogenidgehalt von 4 - 20 Mol-% umfaßt.

9. Lichtempfindliches Aufzeichnungsmaterial nach Anspruch 8, dadurch gekennzeichnet, daß der mittlere Silberhalogenidgehalt 5 - 15 Mol-% beträgt.

10. Lichtempfindliches Aufzeichnungsmaterial nach Anspruch 3, dadurch gekennzeichnet, daß die Silberhalogenidzwillingskörnchen zwei Zwillingsflächen aufweisen.

11. Verfahren zur Herstellung eines lichtempfindlichen Aufzeichnungsmaterials nach Anspruch 1, dadurch gekennzeichnet, daß die Silberhalogenidkörnchen durch folgende drei Stufen hergestellt werden:
Stufe 1: Ausbilden von Kernkörnchen mit einem Silberjodidgehalt von 0 - 5 Mol-% durch Eintragen einer Lösung eines wasserlöslichen Silbersalzes und einer Lösung eines wasserlöslichen Halogenids in eine wäßrige Schutzkolloidlösung unter Aufrechterhalten des pBr-Werts der Stammlösung bei -0,7 bis 2,0 während mindestens der ersten Hälfte der zur Bildung der Kernkörnchen erforderlichen Zeit;
Stufe 2: Ausbilden monodisperser Impfkörnchen kugelförmiger Zwillingskristalle durch Reifenlassen der Kernkörnchen in Gegenwart eines Silberhalogenidlösungsmittels in einer Menge von 10⁻⁵ bis 2,0 Mol/Mol Silberhalogenid; und
Stufe 3: Züchten der Impfkörnchen durch Eintragen einer Lösung eines wasserlöslichen Silbersalzes und einer Lösung eines wasserlöslichen Halogenids oder derselben in Gegenwart feiner Silberhalogenidkörnchen.

12. Verfahren nach Anspruch 11, dadurch gekennzeichnet, daß der pH-Wert der Stammlösung während der Bildung eines beliebigen Teils von mindestens 30 Vol.-% der Silberhalogenidkörnchen bei 1,5 bis 5,8 gehalten wird.

13. Verfahren nach Anspruch 11, dadurch gekennzeichnet, daß der pBr-Wert in Stufe 1 bei -0,7 bis 1,5 gehalten wird.

14. Verfahren nach Anspruch 11, dadurch gekennzeichnet, daß der Anteil der in den gesamten Kernkörnchen enthaltenen Zwillingskernkörnchen 50% oder mehr beträgt.

15. Verfahren nach Anspruch 14, dadurch gekennzeichnet, daß der Anteil 70% oder mehr beträgt.

16. Verfahren nach Anspruch 15, dadurch gekennzeichnet, daß der Anteil 90% oder mehr beträgt.

17. Verfahren nach Anspruch 11, dadurch gekennzeichnet, daß der Anteil der in den gesamten Impfkörnchen enthaltenen kugelförmigen Impfkörnchen 60% oder mehr beträgt.

18. Verfahren nach Anspruch 17, dadurch gekennzeichnet, daß der Anteil 80% oder mehr beträgt.

19. Verfahren nach Anspruch 14, dadurch gekennzeichnet, daß das Silberhalogenidlösungsmittel mindestens ein unter organischen Thioethern, Thioharnstoffderivaten, Verbindungen mit einer Thiocarbonylgruppe zwischen einem Sauerstoffatom oder einem Schwefelatom oder einem Stickstoffatom, Imidazolderivaten, Sulfitsalzen, Thiocyanatderivaten, Ammoniak, Ethylendiaminderivaten, die mit einer Hydroxyalkylgruppe substituiert sind, substituierten Mercaptotetrazolderivaten, wasserlöslichen Bromiden und Benzoimidazolderivaten ausgewähltes Lösungsmittel ist.

20. Verfahren nach Anspruch 19, dadurch gekennzeichnet, daß das Silberhalogenidlösungsmittel mindestens ein unter organischen Thioethern, Thiocyanatderivaten, Ammoniak und wasserlöslichen Bromiden ausgewähltes Lösungsmittel ist.

21. Verfahren nach Anspruch 20, dadurch gekennzeichnet, daß das Silberhalogenidlösungsmittel eine Kombination aus Ammoniak und einem wasserlöslichen Bromid ist.

22. Verfahren nach Anspruch 11, dadurch gekennzeichnet, daß der pH-Wert und die Temperatur in den Stufen 2 und 3 3 - 13 bzw. 30 - 70°C betragen.

23. Verfahren nach Anspruch 22, dadurch gekennzeichnet, daß der pH-Wert und die Temperatur 6 bis 12 bzw. 30 bis 70°C betragen.

24. Verfahren nach Anspruch 11, dadurch gekennzeichnet, daß der pAg-Wert, die Temperatur und der pH-Wert in Stufe 3 5 bis 11, 40 bis 85°C bzw. 1,8 bis 3,0 betragen.

25. Verfahren nach Anspruch 24, dadurch gekennzeichnet, daß der pAg-Wert, die Temperatur und der pH-Wert 6,0 bis 9,5, 60 bis 80°C bzw. 1,8 bis 3,0 betragen.

## Revendications

1. Un matériau photosensible photographique à l'halogénure d'argent comprenant :
- un support sur lequel se trouvent des couches de composant photographique comprenant :
- au moins une couche d'émulsion photosensible contenant une émulsion monodispersée d'halogénure d'argent consistant principalement en grains d'halogénure d'argent maclés,
caractérisé en ce que les gains d'halogénure d'argent comprennent :
a. un noyau à forte teneur en iodure d'argent ;
b. un rapport des dimensions compris entre pas moins de 1,3 et moins de 2 ;
c. principalement des plans [111] ; et
d. des plans de macle parallèles en nombres pairs en proportion de 50 % ou davantage, en nombre par rapport au nombre de grains maclés totaux.

2. Le matériau photosensible selon la revendication 1, caractérisé en ce que les grains maclés consistent en plans [111] et [110].

3. Le matériau photosensible selon la revendication 2, caractérisé en ce que 60 % ou davantage des grains maclés consistent en plans [111].

4. Le matériau photosensible selon la revendication 3, caractérisé en ce que 70 à 100 % des grains maclés consistent en plans [111].

5. Le matériau photosensible selon la revendication 4, caractérisé en ce que 75 % à 98 % des grains maclés consistent en plans [111].

6. Le matériau photosensible selon la revendication 1, caractérisé en ce que l'émulsion d'halogénure d'argent a un degré de monodispersion de 20 %, voire moins, à condition que le degré de monodispersion soit défini par l'équation suivante:$\text{Degré de monodispersion = (déviation standard de la taille de grain/taille de grain moyenne) x 100}$

7. Le matériau photosensible selon la revendication 6, caractérisé en ce que le degré de monodispersion est de 15 % ou moins.

8. Le matériau photosensible selon la revendication 1, caractérisé en ce que l'émulsion d'halogénure d'argent comprend des grains de bromoiodure d'argent présentant une teneur moyenne en halogénure d'argent de 4 à 20 moles %.

9. Le matériau photosensible selon la revendication 8, caractérisé en ce que la teneur moyenne en halogénure d'argent est de 5 à 15 moles %.

10. Le matériau photosensible selon la revendication 3, caractérisé en ce que les grains d'halogénure d'argent maclés ont deux plans maclés.

11. Un procédé de préparation d'un matériau photosensible selon la revendication 1, caractérisé en ce que l'on prépare les grains d'halogénure d'argent par les trois étapes suivantes :
- Etape 1 : formation de grains nucléaires ayant une teneur en iodure d'argent de 0 à 5 moles % en ajoutant une solution de sel d'argent hydrosoluble et une solution d'halogénure hydrosoluble à une solution colloïdale aqueuse de protection tout en maintenant le pBr de la liqueur mère de -0,7 à 2,0 pendant au moins la première moitié du temps nécessaire à la formation des grains nucléaires ;
- Etape 2: formation de grains d'ensemencement monodispersés de cristaux sphériques maclés par maturation des grains nucléaires en présence d'un solvant de l'halogénure d'argent à 10⁻⁵ à 2,0 moles par mole d'halogénure d'argent ; et
- Etape 3 : croissance des grains d'ensemencement en ajoutant une solution de sel d'argent hydrosoluble et une solution d'halogénure hydrosoluble, ou la même chose en présence de grains fins d'halogénure d'argent.

12. Le procédé selon la revendication 11, caractérisé en ce que le pH de la liqueur mère est maintenu entre 1,5 à 5,8 pendant la formation de toute fraction d'au moins 30 % en volume de grains d'halogénure d'argent.

13. Le procédé selon la revendication 11, caractérisé en ce que le pBr à l'étape 1 est maintenu entre -0,7 et 1,5.

14. Le procédé selon la revendication 11, caractérisé en ce que le rapport des grains nucléaires maclés contenus dans les grains nucléaires totaux est de 50 % ou davantage.

15. Le procédé selon la revendication 14, caractérisé en ce que le rapport est de 70 % ou davantage.

16. Le procédé selon la revendication 15, caractérisé en ce que le rapport est de 90 % ou davantage.

17. Le procédé selon la revendication 11, caractérisé en ce que la proportion de grains d'ensemencement sphériques contenus dans les grains d'ensemencement totaux est de 60 % ou d'avantage.

18. Le procédé selon la revendication 17, caractérisé en ce que le rapport est de 80 % ou davantage.

19. Le procédé selon la revendication 14, caractérisé en ce que le solvant de l'halogénure d'argent est au moins un solvant choisi parmi un thioéther organique, un dérivé de thio-urée, un dérivé comportant un groupe thiocarbonyle entre un atome d'oxygène ou un atome de soufre et un atome d'azote, un dérivé d'imidazole, un sel sulfidique, un dérivé de thiocyanate, l'ammoniac, un dérivé d'éthylènediamine substitué par un hydroxyalkyle, un dérivé de mercaptotétrazole substitué, un bromure hydrosoluble et un dérivé de benzoimidazole.

20. Le procédé selon la revendication 19, caractérisé en ce que le solvant de l'halogénure d'argent est au moins un solvant choisi parmi un thioéther organique, un dérivé de thiocyanate. l'ammoniac et un bromure hydrosoluble.

21. Le procédé selon la revendication 20, caractérisé en ce que le solvant de l'halogénure d'argent est une combinaison d'ammoniac et de bromure hydrosoluble.

22. Le procédé selon la revendication 11, caractérisé en ce que le pH et la température au cours des étapes 2 et 3 sont respectivement de 3 à 13 et de 30 à 70°C.

23. Le procédé selon la revendication 22, caractérisé en ce que le pH et la température au cours des étapes 2 et 3 sont respectivement de 6 à 12 et de 30 à 70°C.

24. Le procédé selon la revendication 11, caractérisé en ce que le pAg, la température et le pH au cours de l'étape 3 sont respectivement de 5 à 11, de 40 à 85°C et de 1,8 à 3,0.

25. Le procédé selon la revendication 24, caractérisé en ce que le pAg, la température et le pH sont respectivement de 6,0 à 9,5, 60 à 80°C et de 1,8 à 3,0.
